

## UNITED STATES PATENT OFFICE

2,687,944

## MANUFACTURE OF WATER-SOLUBLE TEXTILE AND OTHER MATERIALS

Edgar Bert Johnson and John Frederick Webster,  
Spondon, near Derby, England, assignors to  
British Celanese Limited, a corporation of Great  
Britain

No Drawing. Application February 9, 1950,  
Serial No. 143,348

Claims priority, application Great Britain  
February 23, 1949

8 Claims. (Cl. 18—54)

1

This invention relates to the manufacture of textile and other materials having a basis of a water-soluble cellulose ether.

It is well known that, for certain purposes, there is a demand for fibres and yarns that can be dissolved by water, and it is an object of the present invention to provide a practical method of making such fibres and yarns from water-soluble cellulose ethers and especially from water-soluble methyl cellulose.

According to the invention, filaments and like articles are made by extruding a spinning solution of a water-soluble cellulose ether in a solvent mixture consisting of water and a water-miscible organic liquid or liquids into a coagulating bath consisting essentially of an organic liquid or liquids miscible in all proportions with the mixture of water and an organic liquid or liquids used as the solvent in the spinning solution.

According to the preferred form of the invention, filaments are made by extruding a solution of a water-soluble cellulose ether, especially a water-soluble methyl cellulose, in aqueous acetic acid into an acetone coagulating bath. The concentration of the acetic acid should be between about 60% and 80% by volume; the concentration of the methyl cellulose in the solution may be about 15%—25% and especially in the neighbourhood of 20%. The acetone may, if desired, be employed in admixture with other liquids, e. g. with up to an equal weight of ethyl alcohol and/or with a smaller proportion, say up to about 10% of its weight, of glycerol; but the best results are obtained using substantially pure acetone or acetone containing up to about 5% or 7% of water. Preferably both the spinning solution and the coagulating bath are at about room temperature, although either or both can be at a higher or lower temperature if desired.

The tenacity of filaments so produced may be increased by stretching them, either individually or grouped together to form yarns, for example by 35%, 50%, 75% or more of their original length. Preferably the filaments are stretched immediately after they have left the coagulating bath and while they are still wet therewith; thus on leaving the bath, the filaments may be passed in succession round two rollers, the second of which runs at a suitably higher peripheral speed than the first. Alternatively or in addition, the filaments may be stretched in the coagulating bath, or they may at some later stage be softened, e. g. by heating to about 290°—310° C., and stretched.

2

The primary advantage of the use of aqueous acetic acid solutions of the methyl cellulose as described is that it enables water-soluble yarns of good dry tenacity to be obtained; thus yarns comprising unstretched filaments may have a tenacity in the neighbourhood of 1.0 gm. per denier and yarns comprising stretched filaments may have a tenacity about 1.25 gm. per denier; these tenacities cannot even be approached by spinning simple aqueous solutions of the methyl cellulose, for example into concentrated aqueous salt solutions or into water-miscible organic liquids such as ethyl alcohol or acetone with or without a small proportion of glycerol. A secondary but not unimportant advantage is, as we have found, that it is considerably easier to dissolve water-soluble methyl cellulose in the aqueous acetic acid to give a solution substantially free from gels and fibrous aggregations and suitable for spinning than it is to dissolve the methyl cellulose in water to give an equally satisfactory solution. It is common knowledge that, to obtain a clear aqueous solution of methyl cellulose within a reasonable time, it is generally necessary to adopt some special expedient; usually the methyl cellulose is first immersed in and thoroughly wetted with hot water (in which it is ordinarily actually insoluble) and the mixture is then cooled while stirring. In contrast to this we have found that water-soluble methyl cellulose can readily be dissolved in the aqueous acetic acid at ordinary temperatures, for example by stirring or by grinding in a ball mill or like device, and that the solutions so obtained are quite satisfactory for spinning.

The invention is illustrated by the following example:

*Example*

40 A water-soluble methyl cellulose of methoxyl content 28.0% and viscosity 15.3 cps. (measured in 2% aqueous solution at 20° C.) was mixed with 70% or 80% (by volume) aqueous acetic acid in a corrosion-resistant ball mill to give a solution of concentration about 20%. This solution was filtered through cellulosic tissue and allowed to stand at 40° C. until it had become substantially completely de-aerated; it was then extruded through a jet comprising a number of orifices of diameter 0.08 mm. into a bath of acetone at room temperature, the filaments so formed travelling through the bath for a length of 48 ins. On leaving the bath, the filaments were passed in succession round two positively-driven 55 rollers whereby they were stretched by 50% of

their original length, and were then wound up as yarns. The yarns so produced were substantially completely soluble in water and had a dry tenacity of about 1.25 gm. per denier or more. When the stretching step was omitted, the tenacity was about 0.9-1.1 gm. per denier.

The process specifically described above, in which a solution of water-soluble methyl cellulose in aqueous acetic acid is extruded into a coagulating bath of acetone, is the preferred method of putting our invention into practice. It can, if desired, be modified in different ways. For example, the acetic acid can be replaced by another water-miscible organic liquid, which preferably contains one or more oxygen atoms and which has a similar or lower solvent power for the methyl cellulose or which by itself is incapable of dissolving the methyl cellulose. For instance the acetic acid may be replaced by another lower fatty acid, e. g. propionic acid; by a hydroxy compound, especially a normally liquid alcohol, e. g. methyl or ethyl alcohol; by a normally liquid hydroxy-ether, e. g. the monoethyl or other lower alkyl mono-ether of ethylene glycol; or by a normally liquid cyclic ether, e. g. dioxane; thus a spinning solution in which the methyl cellulose is dissolved in a 70%-90% aqueous methyl or ethyl alcohol may be used. If desired two or more of the water-miscible liquids may be employed. Moreover, the acetone coagulating bath may be partly or wholly replaced by another lower aliphatic ketone such as methyl ethyl ketone or diethyl ketone, by an alcohol, especially a normally liquid aliphatic alcohol containing 5 or more carbon atoms and especially 7-10 carbon atoms, e. g. octyl alcohol, by a normally liquid hydroxy-ether, or by two or more of these compounds. References to "lower" compounds or radicles are to be understood as denoting compounds or radicles containing not more than 5 carbon atoms.

Although the invention has been described with particular reference to the production of filaments and yarns from a water-soluble methyl cellulose, it may also be applied to the production of filaments and yarns from other water-soluble cellulose ethers, e. g. hydroxyethyl cellulose, carboxymethyl cellulose, or a mixed ether such for instance as hydroxyethyl ethyl cellulose or hydroxyethyl methyl cellulose. It is also of use in the production of two-dimensional shaped articles such as films and foils from the water-soluble cellulose ethers.

Having described our invention, what we desire to secure by Letters Patent is:

1. Process for the production of water-soluble filaments and films, which comprises extruding a spinning solution of a water-soluble cellulose ether in aqueous acetic acid of concentration 60 to 80% by volume into a coagulating bath consisting essentially of at least one organic liquid selected from the group which consists of aliphatic ketones containing at most 5 carbon atoms in the molecule, normally liquid aliphatic alcohols containing 5 to 10 carbon atoms in the molecule, and normally liquid hydroxy-ethers.

2. Process for the production of water-soluble filaments and films, which comprises extruding a spinning solution of a water-soluble methyl cellulose in aqueous acetic acid of concentration 60 to 80% by volume into a coagulating bath consisting essentially of at least one organic liquid

selected from the group which consists of aliphatic ketones containing at most 5 carbon atoms in the molecule, normally liquid aliphatic alcohols containing 5 to 10 carbon atoms in the molecule, and normally liquid hydroxy-ethers.

3. Process for the production of water-soluble filaments and films, which comprises extruding a spinning solution of a water-soluble cellulose ether in an aqueous acetic acid of a concentration 60 to 80% by volume into a coagulating bath consisting essentially of a lower aliphatic ketone.

4. Process for the production of water-soluble filaments and films, which comprises extruding a spinning solution of a water-soluble methyl cellulose in aqueous acetic acid of concentration 60 to 80% by volume into a coagulating bath consisting essentially of acetone and containing 0 to 7% of water.

5. Process for the production of water-soluble filaments and films, which comprises extruding a 15 to 25% solution of a water-soluble methyl cellulose in aqueous acetic acid of concentration 60 to 80% by volume into a coagulating bath consisting essentially of acetone and containing 0 to 7% of water.

6. Process for the production of water-soluble filaments and films, which comprises extruding a spinning solution of a water-soluble cellulose ether in an aqueous acetic acid of a concentration 60 to 80% by volume into a coagulating bath consisting essentially of a lower aliphatic ketone and stretching the products while still wet with the coagulating bath.

7. Process for the production of water-soluble filaments and films, which comprises extruding a spinning solution of a water-soluble cellulose ether in an aqueous acetic acid of a concentration 60 to 80% by volume into a coagulating bath consisting essentially of a lower aliphatic ketone and subsequently stretching the products while softened by heat.

8. Process for the production of water-soluble filaments and films, which comprises extruding a spinning solution of a water-soluble methyl cellulose in aqueous acetic acid of concentration 60 to 80% by volume into a coagulating bath consisting essentially of acetone and containing 0 to 7% of water and subsequently stretching the products while they are softened by being heated to a temperature between 290 and 310° C.

#### References Cited in the file of this patent

#### UNITED STATES PATENTS

| Number    | Name                 | Date          |
|-----------|----------------------|---------------|
| 2,025,730 | Dickie et al. -----  | Dec. 31, 1935 |
| 2,134,895 | Seymour et al. ----- | Nov. 1, 1938  |
| 2,147,640 | Dickie et al. -----  | Feb. 21, 1939 |
| 2,163,723 | Whitehead -----      | June 27, 1939 |
| 2,218,029 | Hubert et al. -----  | Oct. 15, 1940 |
| 2,308,141 | Alles -----          | Jan. 12, 1943 |
| 2,341,586 | Alles -----          | Feb. 15, 1944 |
| 2,350,161 | Gloor -----          | May 30, 1944  |
| 2,495,767 | Reid et al. -----    | Jan. 31, 1950 |

#### FOREIGN PATENTS

| Number  | Country             | Date          |
|---------|---------------------|---------------|
| 508,547 | Great Britain ----- | June 30, 1939 |

#### OTHER REFERENCES

Worden, "Technology of Cellulose Ethers" (1933), V. 3, pages 1305 to 1308.